

(No Model.)

J. R. KINSLEY.

MOLD FOR MAKING WHITE METAL CASTINGS.

No. 309,629.

Patented Dec. 23, 1884.

Fig. 1.



Fig. 2.



Witnesses:

J. W. Browne

O. P. Saylor

Inventor:

John R. Kinsley

# UNITED STATES PATENT OFFICE.

JOHN R. KINSLEY, OF CINCINNATI, OHIO.

## MOLD FOR MAKING WHITE-METAL CASTINGS.

SPECIFICATION forming part of Letters Patent No. 309,629, dated December 23, 1884.

Application filed March 22, 1884. (No model.)

*To all whom it may concern:*

Be it known that I, JOHN R. KINSLEY, a citizen of the United States, residing at Cincinnati, in the county of Hamilton and State of Ohio, have invented a new and useful Improvement 5 in Molds for Making White-Metal Castings, (and according to my knowledge and belief the same has not been in public use or on sale in the United States for more than two 10 years prior to this application,) of which the following is a specification.

My invention relates to an improvement in molds for making white-metal castings, for hinge-tips and other purposes, with wooden 15 cores. The wooden core is covered with a non-inflammable paint or wash, and has a vent from its top down through the center, and also continuing through the pin in the mold on which the core stands and out through 20 the bottom of the mold, the top opening of the vent being covered by a hood, which is formed by projections from the two sides of the mold, which, when closed, come together and form this hood, which prevents the molten metal 25 from entering this vent, whereby the blowing which causes imperfect castings is prevented, and this non-inflammable coating also greatly reduces the smoke and steam by which this blowing is caused, said mold being made of 30 iron or steel, and said wash or paint being composed of one pound of molding-sand, one-fourth pound of pulverized rosin, and one-fourth pound of wheat-flour, mixed thoroughly with water to a stiff paint or paste 35 and applied with a brush to the wooden core, and then thoroughly dried in an oven or otherwise before using.

Figure No. 1 shows the combination complete, and Fig. No. 2 shows a section of the wooden 40 core and pin on which it rests.

In Fig. No. 1, A shows the base of the mold; B B, the two sides of the mold; C, the hinge connecting these two sides. D shows the wooden core in position on the pin of the mold. E shows the pin on which the core stands. F 45 shows the guide-pin or stop which causes the two sides of the mold to come together correctly. G G show the two sides of the mold-cavity. H H show the two shoulders or projections which, coming together, form the 50 hood or vent-cover. I I show the mold-cavities for the gate through which the molten metal is poured. K shows the arm of the lock by which the two sides are fastened together during casting.

In Fig. No. 2, D shows a section of the wooden core. E shows a section of the pin on which said core stands. L shows the longitudinal vent-orifice, open at the top and extending continuously down through the wooden core 60 and pin on which it stands, and out through the bottom of the mold.

The white-metal which I use is composed of one hundred (100) pounds of lead, twenty (20) pounds of antimony, and five (5) pounds 65 of block-tin; but I do not confine myself to the use of any particular metal; therefore

I claim—

The combination of a covered or prepared wooden core, having a longitudinal vent-orifice open at the top, with a mold having a vent communicating therewith, and having a hood in its mold-cavity over the vent-opening in the core, substantially as described, and for the purpose set forth.

JOHN R. KINSLEY.

Witnesses:

O. P. CAYLOR,  
F. W. BROWNE.